# EUROPEAN PATENT SPECIFICATION

(11) **EP 0 018 083 B1**
(45) Date of publication and mention of the grant of the patent: **20.02.1985**
(21) Application number: 80300809.3
(22) Date of filing: 18.03.1980
(51) Int. Cl.: C23F 11/08

(54) **Corrosion inhibitor method for the treatment for boiler water**
Verfahren zur Korrosionshemmung in Heizkesseln
Procédé pour inhiber la corrosion dans des chaudières

(30) Priority: 02.04.1979 US 26273
(43) Date of publication of application: 29.10.1980
(73) Proprietor: BETZ EUROPE, INC., Trevose Pennsylvania 19047 (US)
(72) Inventor: Schuck, Joseph John, Holland Pennsylvania 18966 (US); Godlewski, Irene Theresa, Cinnaminson New Jersey 08077 (US)
(74) Representative: McCall, John Douglas

## Description

Boilers using demineralized makeup water are known to be prone to caustic attack. High pressure boilers are particualrly susceptible to this type of metal corrosion.

The inside surfaces of the boiler are typically protected with magnetite. Hydroxide ion, being the predominant anion in high purity boiler water, can dissolve the magnetite when highly concentrated. Even though high purity water is being used, caustic can nonetheless become highly concentrated, primarily due to the presence of iron oxide deposits on radiant wall tubes. While the bulk water may contain only 5-10 ppm of caustic, it is quite possible to have localized caustic concentrations of up to 100,000 ppm. The iron oxide deposits are extremely porous so that water is drawn thereinto. Due to heat being applied from beneath, steam is generated and passes out of the porous deposit, while fresh water is again drawn thereinto. The result is the noted high concentrations of caustic which must be dealt with if the boiler is to properly be protected.

A widely used method for controlling caustic corrosion in boilers using demineralized (high purity) makeup water, particularly in high pressure boilers, is the coordinated phosphate/pH control treatment. This method of treatment is detailed in an article by George Gibson entitled "The Basics of Phosphate-pH Boiler Water Treatment", Power Engineering, February, 1978, p. 66, which article is incorporated herein by reference to the extent necessary to complete this disclosure. In any event, portions are excerpted below for purposes of explanation.

The coordinated phosphate/pH corrosion control treatment is based on two principles: first, that sodium phosphates are a pH buffer; and second, that disodium hydrogen phosphate converts potentially corrosive caustic into relatively harmless trisodium phosphate according to the following equation: Accordingly, general corrosion is prevented through the control of boiler water pH, and adherent deposits with concomitant caustic corrosion are prevented by maintaining a disodium hydrogen phosphate residual in the boiler water to react with caustic according to equation (1).

The program is implemented with a control chart such as in Figure 1. Disodium hydrogen phosphate is present if the coordinate of pH and phosphate lies within the control boundry.

Many sodium phosphates are used in boiler water treatment. Of these, orthophosphates are preferred. Complex phosphates, in the form of polymer chains, break down into orthophosphates at boiler water temperatures by a process known as reversion. The orthophosphates are monosodium dihydrogen phosphate (MSP), disodium hydrogen phosphate (DSP) and trisodium phosphate (TSP).

Orthophosphates can be identified by name, formula or sodium-to-phosphate ratio which can be expressed with the notation "NA:P0₄", read as sodium-to-phosphate ratio.

Monosodium dihydrogen phosphate has one mole of sodium per mole of phosphate. Therefore, the sodium-to-phosphate ratio is one-to-one (Na:P0₄ = 1: 1). Disodium hydrogen phosphate, with two moles of sodium per mole of phosphate, has a Na:P0₄ = 2:1, and trisodium phosphate has a Na:P0₄ = 3:1.

Sodium-to-phosphate ratios are useful to describe mixtures of phosphates in solution. For example, solutions of DSP and TSP have a Na:P0₄ between 2:1 and 3:1. The Na:P0₄ is fairly proportional to the mix ratio. For instance, a solution of half DSP and half TSP a ratio of about 2.5:1 (it is actually 2.46:1 because DSP and TSP have different molecular weights).

Figure 2 shows the relation between solution pH and phosphate concentration for various sodium-to-phosphate molar ratios. Examination of the figure reveals pH increases with increasing Na:P0₄ (at equal phosphate concentrations). Acordingly, solution pH and phosphate concentration identify phosphate form, it being kept in mind that disodium hydrogen phosphate is the species which neutralizes caustic according to equation (1).

A trisodium phosphate solution exists if the phosphate/pH coordinate falls on the Na:P0₄ = 3:1 line; disodium hydrogen phosphate solution if the coordinate falls on the 2:1 line; and a mixture of DSP and TSP if the coordinate falls between the 2:1 and 3:1 lines. As the coordinate approaches the 3:1 line, there is more and more TSP and less and less DSP in the solution.

The solution is a mixture of TSP and caustic if the coordinate falls above the 3:1 line. In this "free caustic" region there is no DSP to tie up the caustic.

It is seen that the phosphate/pH coordinate must be below the Na:P0₄ = 3:1 line to ensure that there is DSP in solution to tie up the caustic. The further the phosphate/pH coordinate is kept below the line the greater the caustic-absorbing capacity of the water and the less chance of drifting into the region above the 3:1 line.

Figure 2 is based on pure sodium phosphate solution. The pure solution theory can be used with impure boiler water because the concentration of other species is low and their solubility high. Complex chemistry is avoided by using pH as a variable. It is desirable to keep the Na:P0₄ between 2.8:1 and 2.2:1. The phosphate-pH control chart, Figure 1, is a refinement of Figure 2 with a control boundary in the appropriate range to prevent caustic corrosion. The control chart is the heart of phosphate-pH control.

There has been some confusion in applying sodium-to-phosphate ratios. The NA:P0₄ used in phosphate-pH control is determined only from boiler water pH and phosphate concentration, not by measuring sodium and phosphate concentrations of the boiler water.

This information can be used to make a phosphate-pH control chart by first setting phosphate limits. Maximum allowable phosphate decreases with increasing boiler pressure because of carryover and phosphate "hideout". The latter term, incidentally, refers to the phenomenon of diminishing boiler water phosphate levels with increased firing rate (everything else held constant) and the reappearance of boiler water phosphate level when the firing rate is reduced. Hideout phosphate is believed to be caused by precipitating the phosphates under high heat flux conditions.

Individual plants have set their own phosphate limits, based on what works for them and on results at similar installations. The limits chosen for the control chart shown in Figure 1 are consistent with industry practice and have provided to be satisfactory in practical applications.

Note that the residual phosphate limits contained in the control chart (Figure 1) are the maximum levels recommended for satisfactory boiler operation. Whatever the allowable residual phosphate concentration, it is prudent to operate with as little phosphate as practicable.

There should preferably be an upper Na:P0₄ limit of 2.85:1 to prevent caustic corrosion and preferably a lowre Na:P0₄ limit of 2.13:1 to prevent acid attack. But, it would be prudent to include a safety factor into these numbers, which safety factor depends on individual boiler characteristics and system water tightness. Lower pressure boilers have less trouble with caustic corrosion than higher pressure boilers and generally can be run with Na:P0₄ close to the 2.85:1 line. Of course, if caustic corrosion is occurring a lower maximum limit should be set for the boilers involved. High pressure boilers tend to be more susceptible to caustic corrosion, and a maximum Na:P0₄ line of 2.6:1 usually is chosen. This has provided to be an effective limit.

It should be understood from the foregoing that the coordinated phosphate/pH control treatment consists primarily of two basic steps as follows:
(1) maintenance of an appropriate level of residual orthophosphate in the boiler water; and
(2) maintenance of the proper Na:P0₄ ratio in the water.

The residual orthophosphate level will depend on such known factors as the nature and severity of the problem and boiler pressure. Since it is considered best to operate with as little phosphate as possible, amounts as low as about 1 ppm could be used, with about 2 ppm being the preferred minimum. While amounts as high as about 50 ppm residual orthophosphate could be used, about 30 ppm is the preferred maximum.

While the coordinated phosphate/pH corrosion control treatment is widely used, it is not without its drawbacks and limitations. Often, it is desirable to supplement the treatment with additional corrosion inhibitor; however, this is not always practible. It has been customary for many years to use the sodium salt of a polymeric dispersant, such as sodium polymethacrylate, as the supplement. When the sodium salt form is used, the Na:P0₄ in the boiler water is often significantly altered and the solids level of the boiler water rises. If the Na:P0₄ is allowed to rise over the 3:1 line of Figure 2, caustic attack again becomes a problem, and, particularly in high pressure boiler systems, increased solids levels can lead to undesirable foaming in the water. Thus, the use of supplemental treatment has been severely limited. In fact, when the Na:P0₄ is near the control limit, the supplemental treatment has been completely omitted.

The present invention relates to an improvement in the coordinated phosphate/pH corrosion treatment for boiler water. According to the present invention, a supplemental corrosion inhibitor is provided which neither significantly alters the sodium burden of the boiler nor significantly increases the solids level therein.

The present invention is drawn to the use, in conjunction with a coordinated phosphate/pH corrosion control treatment, of an aqueous solution of an organic acid dispersant which has been neutralized with ammonia °2 any one of a class of specific amines, hereinafter referred to as "alpha" amines. More specifically, according to the present invention, the organic acid dispersant is neutralized with a suitable amine (or NH₃) which is volatile under the conditions of the boiler water to be treated and has a basicity constant of 8.0 or less. A detailed description of how to determine suitbale amines is presented below.

The invention offers certain advantages as follows:
(1) the sodium burden in the boiler is limited, thus limiting caustic gouging and other forms of boiler metal corrosion;
(2) advantage (1) is accomplished with volatile materials that do not concentrate in the boiler and, thereby, do not contribute to either corrosion or deposition processes; and
(3) the supplemental material will aid in corrosion control in both the boiler and in the steam distribution system (due to volatile neutralizing agents).

The utility of the present invention is considered to be greatest for those high pressure (above 900-1200 psig i.e. above 6205.5-8274 KPa gauge) boiler systems experiencing difficulty in maintaining a Na:P0₄ (ess than 2.8:1. The use of a low sodium supplement under these conditions does not contribute to the sodium burden of the boiler, thereby simplifying the maintenance of a coordinated phosphate/pH control treatment, i.e., supplemental feed to the boiler feedwater can be made without disrupting the sodium to phosphate ratio.

According to the present invention, a supplemental corrosion inhibitor is provided in which a volatile organic base has replaced caustic as a neutralizing agent. This resulting alkaline product is considered to be preferable to an acidic product. Furthermore, the volatile organic base finds utility as a condensate corrosion inhibitor, neutralizing carbonic acid at steam condensation sites.

### The Organic Acid

Any reference hereinafter to the polymers used in accordance with the present invention is intended to include the polymers individually as well as any combination of homopolymer, copolymer and mixtures thereof. The term "polymeric acid" is intended to include any polymer containing acid functional group(s), as well as acid precursor compounds (e.g., anhydrides).

As already noted, the compounds which are considered to be useful in practicing the present invention are any of the well known organic acid dispersants, such as polymeric sulfonic acids, polymeric phosphonic acids, polymeric carboxylic acids and poly phdsphonic acids.

Illustrative examples of polymeric carboxylic acids would be as follows:
polyacrylic acid
polymethacrylic acid
polymaleic anhydride
acrylic acid/hydroxypropylacrylate copolymer
sulfonated styrene/maleic anhydride copolymer
methylvinyl ether/maleic anhydride copolymer
acrylic acid/methacrylic acid copolymer

Illustrative examples of polymeric sulfonic acids would be as follows:
sulfonated polystyrene
polyvinylsulfuric acid
sulfonated styrene/maleic anhydride copolymer
polyvinylsulfonic acid
poly[2-acrylamido-2-methylpropanesulfonic acid]

Illustrative examples of poly phosphonic acids would be:
ethylenediamine tetra(methylene phosphinic acid)
1-hydroxyethylidene-1,1-diphosphonic acid
nitrilotri(methylene phosphonic acid)

These compounds are believed to be useful in boilers of up to about 1500 psig (10,342.5 K Pa gauge).

The polymeric phosphonic acids are believed to be suitable for use at pressures up to well above 1500 psig (10,342.5 K Pa gauge). However, few are presently commercially available. Illustrative examples of these compounds are polyvinyl phosphonic acid and its substituted analogs.

As is well known in the art, the amount of supplemental corrosion inhibitor would depend on such factors as the nature and severity of the problem to be treated and could vary over a wide range. The amount of neutralised organic acid used as supplemental corrosion inhibitor could, accordingly, be as low as about 1 part polymer per million parts of boiler water (ppm). The preferred minimum is considered to be about 5 ppm. Based on economic considerations, the upper limit for the neutralized organic acid dosage is considered to be about 150 ppm; while 50 ppm represents the preferred maximum.

With respect to the polymeric organic acids, it is well known that molecular weight is not critical. In any event, a molecular weight of from about 1000 to about 200,000 is believed to be operable.

### The Neutralizing Agent

Suitable compounds for use as neutralizing agents in accordance with the present invention have already been described as ammonia and alpha amines. The important properties of these compounds are, first, that they are volatile under the operating conditions of the boiler and, second, that they have sufficient basicity to neutralize the organic acid dispersant. Defining the first property in terms of distribution ratio and the second in terms of basicity constant, pKₜ, alpha amines are those having a distribution ratio of 0.01 or greater under the operating conditions of the boiler and a pK_{b} of 8.0 or less.

The distribution ratio, DR, is defined as the quantity of volatile amine found in the stream phase over the quantity found in the bulk fluid and is represented by: The values for this ratio, of course, are easily obtained by drawing a condensed steam sample and a blowdown sample from the boiler and analyzing for respective amine contents.

The basicity constant is a well known comparison for basicities of amines in terms of their respective abilities to accept hydronium ion from water. Using the reaction: the basicity constant, pK_{b}, is defined by: Each amine has its own pK_{b}, and, the lower the value, the stronger the base. As is well known to the artisan, tabulated values for pK_{b}'s are readily obtainable from numerous chemical reference books. For example, a table of such values can be found in the "Handbook of Chemistry and Physics", The Chemical Rubber Co., 45th Edition (1964-1965), p. D-76.

Following is an exemplary list of alpha amines believed to be suitable for use in accordance with the present invention:
morpholine
aminomethylpropanol (AMP)
dimethylaminomethylpropanol (DMAMP)
cyclohexylamine
dimethylpropanolamine (DMPA)
diethylaminoethanol
N-hexylamine
methoxypropylamine (MPA)
benzylamine
monoisopropanolamine
1,6 hexanediamine
1,3 diaminopropane
tributylamine
triethylamine
n-amylamine
n-methylmorpholine
N,N-dimethyl-1,3-propanediamine.

### EXAMPLES

### Determining Distribution Ratios

### Example 1

A first series of tests were conducted to determine the DR's of various compounds using a research boiler similar to the one schematically illustrated in Figure 3. Two fiberglass feed tanks were filled with a total of 600 liters of deionized water which was deaerated by nitrogen sparging for two hours. At the end of the deaeration period one tank was charged with 50 ppm ammonia or alpha amine, while the other was charged with various chemicals to provide boiler test water as follows:
"P" alkalinity = 200 ppm
residual silica = ₂₀ ppm, added as sodium metasilicate
residual phosphate = 20 ppm, added as sodium dihydrogen phosphate
residual sulfite = 20 ppm, added as sodium sulfite
calcium hardness = 10 ppm, added as calcium chloride
magnesium hardness = 5 ppm, added as magnesium sulfate
cycles of concentration = 15 ppm
O2 level after N₂ sparging = 0.25-0.5 ppm

The boiler was energized and allowed to come to equilibrium overnight at 100 psig (689.5 KPa gauge). On the second through fifth days two sets of samples (each set consisted of a steam sample and a blowdown sample) were taken per pressure step at a minimum of one hour and a maximum of one and a half hours between sets (at a given pressure). The samples, refrigerated during the accumulation stage in glass containers, were then analyzed using standard gas chromatographic procedures under the following conditions:
G.C. unit: Perkin Elmer Model 990
Detector(s): Thermal conductivity or flame ionization
Column Size: 6' (1.829 m) x 2 mm id Pyrex
Packing: 14% Carbowax 20 M/2% KOH on 80/1.00 mesh Supelcoport Oven Temperature: 110°C
Carrier Gas: N₂ at 20 ml/min at 40 psig (275.8 KPa gauge)
Sample Size: 1 µl
Injection Temperature: 105°C.

The resulting distribution ratios, calculated according to equation (I), are reported below in Table 1. Also reported are the dissociation constants, pK_{b}, for the materials tested.

### Example 2

An investigation was undertaken to determine the possible effects, if any, of boiler chemicals or water quality on DR. The testing method used was similar to that reported in Example 1. In the present test, however, water "P" alkalinity was increased by a factor of two; and in the comparative "without chemical" tests, the hardness, phosphates and silicates were removed. completely. Some results of these tests are reported below in Table 2 in terms of comparative average DR values with chemicals and without chemicals. All DR's reported are averages of at least two to nine separate data points.

The results of Table 2 are seen to indicate that over the pressure range of interest, with respect to practicing the present invention, no significant effect on DR was noted due to either the absence of boiler chemicals or an increase in alkalinity.

### Example 3

Also investigated was the effect, if any, of increased neutralizing agent concentration on the various DR's. This was accomplished by simply doubling the concentration from 50 ppm to 100 ppm and comparing the results. A testing method similar to that reported in Example 1 was used. The compounds tested were morpholine and cyclohexylamine. The results of these tests are reported below in Table 3 in terms of comparative average DR at 50 ppm and 100 ppm.

Based on the results from Table 3, there is seen to be no significant effect of concentration on the DR. Of course, the individual values for quantity of test compound in the steam and blowdown samples increased significantly, but the magnitude of the DR still remained about the same.

### Making Neutralized Organic Acid

### Example 4

This example is seen to illustrate the preparation of an aqueous solution of neutralized organic acid to be used in accordance with the present invention. The starting material was polymethacrylic acid (PMA) having the formula. which polymer had a molecular weight average of 6,000 to 12,000 as determined by gel permeation chromatography, using as reference a commercial sodium polymethacrylate of advertised molecular weight of 8,000-10,000.

A stock solution is made by the following procedure:
1. weigh out 250 g of tap water (pH = 8.2)
2. add 65 g of PMA (30.8% actives)
3. mix well
4. record pH and neutralize to desired pH with amine

At this point, the 4% PMA solution is reweighed and the amount of neutralizing agent used is recorded. The solution is brought to a final weight of 500 g and a final pH reading is taken. The tap water added increased the pH by about .2 units.

The weights of the neutralizing agent used to reach various pH's for numerous solutions actually made were as follows:
Solution 1: 4% PMA stock solution, 500 g total weight, pH about 2.5
Solution 2: Solution 1 neutralized to pH = 7 with 17.5 g of morpholine; final pH = 7.2
Solution 3: Solution 1 neutralized to pH = 7 with 18.0 g of AMP; final pH = 7.1
Solution 4: Solution 1 neutralized to pH = 7 with 17.2 g of cyclohexylamine; final pH = 7.0
Solution 5: Solution 1 neutralized to pH = 9.5 with 211.3 g of morpholine; final pH = 9.7 (this solution less than 4% PMA)
Solution 6: Solution 1 neutralized to pH = 10 with 25.5 g of AMP; final pH = 10.0
Solution 7: Solution 1 neutralized to pH = 7 with 15.5 g of morpholine, then to pH = 10.8 with 59.7 g of AMP; final pH = 10.9
Solution 8: Solution 1 neutralized to pH = 7 with 18.2 g of morpholine, then to pH = ₁₀.₉ with 53.7 g of cyclohexylamine; final pH = 11.1
Solution 9: Solution 1 neutralized to pH = 7 with 18.4 g of morpholine, then to pH = 9.8 with 46.8 g of AMP; final pH = 10.1
Solution 10: Solution 1 neutralized to pH = 19.0 g of morpholine to pH = 9 with 11.1 g of AMP, then to pH = 11 with 37.9 g of cyclohexylamine; final pH = 11.0
Solution 11: Solution 1 neutralized to pH = 7 with 24.1 g of morpholine, to pH = 9 with 15.3 g of AMP, then to pH = 11 with 8.9 g of sodium hydroxide anhydrous; final pH = 11.5
Solution 12: Solution 1 neutralized to pH = 8 with 21.2 g of morpholine; final pH = 8.0
Solution 13: Solution 1 neutralized to pH = 7.5 with 22 g of AMP; final pH = 8.0
Solution 14: Solution 1 neutralized to pH = 8 with 20.9 g of cyclohexylamine; final pH = 8.1

### Example 5

This example is seen to further illustrate the preparation of an aqueous solution of neutralized organic acid to be used in accordance with the present invention. The starting material was Acrysol A-41, commercially available from Rohm and Haas. It is a copolymer of methacrylic and acrylic acid, having a molecular weight average of about 10,000-12,000 and a mole ratio of methacrylic acid to acrylic acid of about 9:1.

A stock solution is made according to the same procedural steps set forth in the preceding example, however, (71.5 g of) Acrysol A-41 (28% actives) was used instead of the PMA.

The weights of the neutralizing agent used to reach various pH's for numerous solutions actually made were as follows:
Solution 1: 4% copolymer stock solution, 500 g total weight, pH about 2.65
Solution 2: Solution 1 neutralized to pH = 7 with 19.3 g of morpholine; final pH = 7.2
Solution 3: Solution 1 neutralized to pH = 7 with 20.2 g of AMP; final pH = 7.2
Solution 4: Solution 1 neutralized to pH = 7 with 23 g of cyclohexylamine; final pH = 7.6
Solution 5: Solution 1 neutralized to pH = 9.2 with 129.6 g of morpholine; final pH = 9.4 (not stable at this pH)
Solution 6: Solution 1 neutralized to pH = 10 with 43.6 g of AMP; final pH = 10.2
Solution 7: Solution 1 neutralized to pH = 10 with 35.5 g of cyclohexylamine; final pH = 10.1
Solution 8: Solution 1 neutralized to pH = 7 with 21.7 g of morpholine, then to pH = 9 with 13.6 g of AMP, then to pH = 10.8 with 114 g of cyclohexylamine; final pH = 11.1

### Efficacy of Treatment in Boiler

### Example 6

A series of tests were conducted to determine the efficacy of neutralized organic acids as boiler water treatments. The tests were conducted in the research boiler described in Example 1 and schematically illustrated in Figure 3. As already noted, certain boilers are highly susceptible to caustic corrosion as a result of iron oxide deposits formed on interior surfaces. Thus, any treatment which will prevent the formation of iron oxide deposits is considered to be a highly desirable supplement for a coordinated phosphate/pH control program.

Since the research boiler was electrically powered using immersion heated probes, deposits formed directly on probe surfaces. On completion of the tests, the deposits formed on the heating probes were analyzed to determine the quantity of iron oxide present and the total amount of deposit.

During the tests performed, boiler conditions included a coordinated phosphate/pH control program, 15 cycles of concentration, operating pressure of 1450 psig (9997.75 KPa gauge), 3.4 ppm Fe'2 contaminated feedwater, and boiler probes of differing heat flux values. One probe had a heat flux value of 240,000 BTU/ft2/h (757,200 W m-²); while the other had a heat flux of 185,000 BTU/ft²/h (583,675 W m-²). Test durations were 2 days.

The feedwater had the following composition:
7.5 ppm NaHC0₃
0.04 ppm Silica
8.2 ppm Tri-sodium phosphate
0.2 ppm antifoam (polyalkylene glycol)
6 ppm NaN0₃ (for conductivity)
16.7 ppm FeS0₄ (3.4 ppm Fe)

The tests included comparative studies of neutralized polymeric acid dispersants with commonly used polymeric acid dispersants as sodium salts. The materials tested were as follows:
Comparative Product X: Commercial sodium polymethacrylate, reported molecular weight = 6,000-8,000
Comparative Product Y: Commercial sodium polymethacrylate, reported molecular weight = 8,000-10,000
Product A: Polymeric acid starting material of Example 5, neutralized with AMP, pH = 10.0, stored at 120°F (48.9°C) for three months before testing
Product B: Polymeric acid starting material of Example 5, neutralized with morpholine, pH = 8.0, stored at 120°F (48.9°C) for three months before testing
Product C: Polymeric acid starting material of Example 4, neutralized with morpholine and AMP, pH = 10.3, stored at 120°F (48.9°C) for three months before testing
Product D: Polymeric acid starting material of Example 4, neutralized with morpholine, pH = ₈.₁, stored at 120°F (48.9°C) for three months before testing

The results of these tests are reported below in Table 4 in terms of amount of iron deposition (in g/ft² and g/m²) on the probes.

Based on the results reported in Table 4, not only are treatments according to the present invention considered to be efficacious for boiler water, but they are seen to compare favourably with treatments containing the sodium salts of the organic acids. Accordingly, the co-ordinated phosphate/pH corrosion control treatment can be supplemented with an organic acid treatment in a form which will neither adversely affect the critical Na:P0₄ nor increase the solids level in the boiler water.

It should be kept in mind that the stronger the basicity of the neutralizing agent according to the present invention, the less of such neutralizing agent is required to neutralize the polymeric acid dispersant. To avoid problems related to fungi growth, higher pH formulations, e.g., above 8.5, are preferred.

A preferred supplemental treatment composition for use with the co-ordinated phosphate/pH corrosion control treatment is Solution 1 of Example 5 neutralized to pH = 8.5 with 27.3 grams of morpholine.

## Claims

1. A co-ordinated phosphate/pH corrosion control method for the treatment of boiler water, in which residual orthophosphate is maintained in the water in an amount of from 1 to 50 ppm, characterised by maintaining the Na:P0₄ ratio in the water at from 2:1 to less than 3:1 and by supplementing the treatment with an amount of an aqueous solution of a reaction product of an organic acid and a neutralizing agent selected from the group consisting of (1) alpha-amines having a distribution ratio of 0.01 or greater under the operation conditions of the boiler and a basicity constant (pKb) of 8.0 or less, and (ii) ammonia, said amount being such as to provide from 1 to 150 parts of the neutralized organic acid per million parts of boiler water being treated, and said organic acid being a member selected from the group consisting of polymeric carboxylic acids, polymeric sulfonic acids, polyphosphonic acids and polymeric phosphonic acids.

2. A method as claimed in claim 1, characterised in that the organic acid is carboxylic acid polymer.

3. A method as claimed in claim 2, characterised in that the organic acid is selected from the group consisting of acrylic acid polymer and methacrylic acid polymer.

4. A method as claimed in claim 3, characterised in that the organic acid is copolymer of acrylic acid and methacrylic acid.

5. A method as claimed in claim 2, characterised in that the organic acid is polymethacrylic acid.

6. A method as claimed in any one of the preceding claims, characterised in that the "alpha" amine is at least one member selected from the group consisting of morpholine, cyclohexylamine and aminomethylpropanol.

7. A method as claimed in any one of the preceding claims, characterised in that the neutralised organic acid is added in an amount of from 5 to 50 ppm.

8. A method as claimed in any one of the preceding claims, characterised in that the Na:P0₄ is maintained at from 2.13:1 to 2.85:1.

9. A method as claimed in claim 9, wherein the Na:P0₄ is maintained at from 2.2:1 to 2.6:1.

10. A method as claimed in any one of the preceding claims, characterised in that the residual orthophosphate level is maintained at from 2 to 30 ppm.

## Patentansprüche

1. Verfahren zur Korrosionshemmung in Heizkesseln durch Einstellung des Phosphatgehaltes und pH-Werts des Kesselspeisewassers, wobei der Restgehalt an Orthophosphat im Wasser bei 1 bis 50 ppm gehalten wird, dadurch gekennzeichnet, daß man im Wasser ein Verhältnis Na:PO₄von 2:1 bis <3:1 einhält und eine wässrige Lösung eines Reaktionsprodukts einer organischen Säure mit einem neutralisierenden Mittel in Form von (A) a-Aminen mit einem Verteilungsverhältnis ?0,01 unter Arbeitsbedingungen des Kessels und pKb:5-:- 8 oder (B) Ammoniak in solcher Menge, daß 1 bis 150 Teile neutralisierte organische Säure auf eine Million Teile Kesselspeisewasser kommen, und man als organische Säure polymere Carbon-, Sulfon- oder Phosphonsäuren oder Polyphosphonsäuren verwendet.

2. Verfahren nach Anspruch 1, dadurch gekennzeichnet, daß man als organische Säure eine Polycarbonsäure verwendet. -

3. Verfahren nach Anspruch 2, dadurch gekennzeichnet, daß man als Säure Polyacryl- oder Polymethacrylsäure verwendet.

4. Verfahren nach Anspruch 3, dadurch gekennzeichnet, daß man als Säure das Copolymere von Acryl-und Methylsäure verwendet.

5. Verfahren nach Anspruch 2, dadurch gekennzeichnet, daß man als Säure Polymethacrylsäure verwendet.

6. Verfahren nach einem der Ansprüche 1 bis 5, dadurch gekennzeichnet, daß man für die a-Amine zumindest eine Verbindung aus der Gruppe Morpholin, Cyclohexylamin und Aminomethylpropanol verwendet.

7. Verfahren nach einem der Ansprüche 1 bis 6, dadurch gekennzeichnet, daß man die neutralisierte Säure in einer Menge von 5 bis 50 ppm zusetzt.

8. Verfahren nach einem der Ansprüche 1 bis 7, dadurch gekennzeichnet, daß man das Verhältnis Na:P0₄ zwischen 2,13:1 und 2,85:1 hält.

9. Verfahren nach Anspruch 8, dadurch gekennzeichnet, daß man das Verhältnis Na:P0₄ zwischen 2,2:1 und 2,6:1 hält.

10. Verfahren nach einem der Ansprüche 1 bis 9, dadurch gekennzeichnet, daß man den Restgehalt an Orthophosphat bei 2 bis 30 ppm hält.

## Revendications

1. Procédé de lutte contre la corrosion dit procédé phosphate/pH coordonnés pour le traitement d'eaux de chaudières et bouilleurs, dans lequel la teneur de l'eau en orthophosphate résiduel est maintenue entre 1 et 50 ppm, procédé caractérisé en ce que l'on maintient dans l'eau le rapport Na:P0₄ entre 2:1 et moins de 3: 1, et en ce que l'on complète le traitement avec une proportion d'une solution aqueuse d'un produit de réaction d'un acide organique avec un agent neutralisant choisi parmi (1) des alpha-amines ayant un rapport de répartition, tel que défini, de 0,01 ou plus dans les conditions de fonctionnement de la chaudière, et une constante de basicité (pKb) de 8,0 ou moins, et (2) l'ammoniac, cette proportion devant donner 1 à 150 parties de l'acide organique neutralisé par million de parties de l'eau à traiter, et l'acide organique étant choisi parmi des acides carboxyliques polymères, des acides sulfoniques polymères, des acides polyphosphoniques et des acides phosphoniques polymères.

2. Procédé selon la revendication 1, caractérisé en ce que l'acide organique est un polymère d'acide carboxylique.

3. Procédé selon la revendication 2, caractérisé en ce que l'acide organique est choisi parmi un polymère de l'acide acrylique ou de l'acide méthacrylique.

4. Procédé selon la revendication 3, caractérisé en ce que l'acide organique est un copolymère de l'acide acrylique et de l'acide méthacrylique.

5. Procédé selon la revendication 2, caractérisé en ce que l'acide organique est un acide polyméthacry- lique.

6. Procédé selon l'une quelconque des revendications précédentes, caractérisé en ce que l' "alpha" amine est la niorpholine, la cyclohexylamine ou l'aminométhylpropanol ou plusieurs de ces amines.

7. Procédé selon l'une quelconque des revendications précédentes, caractérisé en ce que l'acide organique neutralisé est ajouté dans une proportion de 5 à 50 ppm.

8. Procédé selon l'une quelconque des revendications précédentes, caractérisé en ce que le rapport Na:P0₄ est maintenu entre 2,13:1 et 2,85:1.

9. Procédé selon la revendication 9, dans lequel le rapport Na:P0₄ est maintenu entre 2,2:1 et 2,6:1.

10. Procédé selon l'une quelconque des revendications précédentes, caractérisé en ce que la teneur en orthophosphate résiduel est maintenue entre 2 et 30 ppm.
